# EUROPEAN PATENT SPECIFICATION

(11) **EP 0 453 270 B1**
(45) Date of publication and mention of the grant of the patent: **10.04.1996**
(21) Application number: 91303442.7
(22) Date of filing: 17.04.1991
(51) Int. Cl.: H01F 1/053

(54) **Rare-earth based magnetic materials, production process and use**
Seltenerd-basierte magnetische Materialien, Herstellungsverfahren und Anwendung
Matériaux magnétiques à base de terres rares, procédé de fabrication et utilisation

(30) Priority: 18.04.1990 IE 135990; 04.09.1990 IE 320190; 28.02.1991 IE 67191
(43) Date of publication of application: 23.10.1991
(73) Proprietor: THE PROVOST, FELLOWS AND SCHOLARS OF THE COLLEGE OF THE HOLY AND UNDIVIDED TRINITY OF QUEEN ELIZABETH NEAR DUBLIN, Dublin 2 (IE)
(72) Inventor: Coey, John Michael David, Castleknock, County Dublin (IE); Sun, Hong, Dublin 9 (IE)
(74) Representative: Baldock, Sharon Claire

(56) References cited:
- EP-A- 0 470 476
- JP-A-60 131 949
- US-A- 4 402 770
- PATENT ABSTRACTS OF JAPAN, vol. 10, no. 11 (E-374)[2068], 17th January 1986; & JP-A-60 176 202 (HITACHI KINZOKU K.K.) 10-09-1985
- PATENT ABSTRACTS OF JAPAN, vol. 11, no. 117 (E-498)[2564], 11th April 1987; & JP-A-61 263 201 (HITACHI METALS LTD) 21-11-1986
- PATENT ABSTRACTS OF JAPAN, vol. 14, no. 41 (E-879)[3984], 25th January 1990;
- & JP-A-1 274 401 (TDK CORP.) 02-11-1989
- IEEE TRANSACTIONS ON MAGNETICS, vol. 23, no. 5II, September 1987, pages 3098- 3100; S. HIGANO et al.: "Magnetic properties of RE-TM-N system"
- PATENT ABSTRACTS OF JAPAN, vol. 9, no. 310 (E-364)[2033], 6th December 1985; & JP-A-60 144 909 (DAIDO TOKUSHUKO K.K.) 31-07-1985
- NRC HANDELSBLAD, 4th April 1991, NL; "Nieuwe legering ontwikkeld voor permanente magneten"
- A.F.Wells, Structural Inorganic Chemistry, 3rd. edition, page 176;
- Handbook of Magnetic Materials, Coey et. al., Elsevier Science Publishers B.V., 1991, pages 2-4;

## Description

The invention relates to new magnetic materials having improved magnetic properties, to processes for their production and to the use of the new materials to make permanent magnets.

Magnets have many applications in engineering and science as components of apparatus such as electric motors, electric generators, focussing elements, lifting mechanisms, locks, levitation devices, anti-friction mounts and so on. In order for a magnetic material to be useful for making a permanent magnet three intrinsic properties are of critical importance. These are the Curie temperature (Tc) i.e. the temperature at which a permanent magnet loses its magnetism, the spontaneous magnetic moment per unit volume (Mₛ) and the easy uniaxial anisotropy conventionally represented by an anisotropy field Bₐ. The Curie temperature is of particular significance because it dictates the temperature below which apparatus containing the magnet must be operated.

During this century much research has been directed to developing magnetic materials which combine high Curie temperatures and improved magnetic moments with strong uniaxial anisotropy. For many years magnetic materials of the AlNiCo type were used in permanent magnets for practical applications. In the late 1960's it was discovered that alloys of the rare earth elements, particularly samarium when alloyed with cobalt, had magnetic properties which made them superior as permanent magnets to the AlNiCo type. Compounds of samarium and cobalt provided magnets which were particularly successful in many demanding practical applications requiring a magnet with a high energy product. However the high cost of cobalt as a raw material led investigators in the early 1980's to consider the possibility of combining the cheaper and more abundant iron with the magnetically superior rare earth elements to produce permanent magnets with improved magnetic properties. A major breakthrough came in 1983 when the Sumitomo Special Metals Company and General Motors of America independently developed a magnetic material which combined a rare earth element and iron and incorporated a third element, boron, into the crystal lattice to give an intermetallic compound, Nd₂Fe₁₄B which can be used to produce magnets with an excellent energy product, but a lower Curie temperature than the Sm-Co materials. These Nd-Fe-B magnetic materials can have a Curie temperature of up to 320^{o}C and are particularly described in three European applications, EP-A-0101552, EP-A-0106948 and EP-A-0108474. Derivatives of these boride materials represent the state of the art to date in magnet technology. However they are somewhat unstable in air and change chemically, gradually losing their magnetic properties so that despite Curie temperatures in excess of 300^{o}C in practice they are not suitable for operating at temperatures greater than 150^{o}C.

The fact that the incorporation of boron into the crystal lattice of intermetallic materials containing a rare earth element and iron serves to improve magnetic properties has encouraged investigators to search for new compounds of elements other than boron in combination with rare earth elements and iron.

In 1987 Higano et al (IEEE Transactions on Magnetics, vol, Mag-23, No. 5 Sept 1987) reported an attempt to carry out a nitriding reaction by exposure of powders of Sm₂Fe₁₇ alloy to gaseous nitrogen at temperatures of 500 and 1100°C. The experiment was intended to produce a compound of the formula Sm₂Fe₁₇-N which it was hoped would have improved magnetic properties. However Higano et al found no evidence that such a material was produced by this process but instead found that the nitriding process simply decomposed the rare-earth iron alloy starting material to produce iron and nitrides of the rare earth elements.

In Japanese Patent Application No 60-131949 of Hitachi Metals Corporation the production of a material containing iron, praseodymium and nitrogen is described in which an alloy containing Fe and Pr is first prepared by melting iron and praseodymium in the ratio 29.1% wt Pr and 70.9% wt Fe to produce a multiphase product. This multiphase alloy is then heated in ammonia at 500°C. Thereafter the product is sintered at 1100°C for two hours in nitrogen. As is shown herein such a high sintering temperature decomposes any earlier product.

The present inventors have now produced a new magnetic material of improved properties which includes at least a rare earth element, iron and a group VA element with optionally one or more other elements. These materials have Curie temperatures in excess of 400°C. The successful production of these materials is unexpected having regard to the teaching of Higano et al and JP-A-60-131949.

In accordance with one aspect of the invention there is provided a magnetic material of the general formula:

RₓFe_{y}X'ₐZ_{b}

which has a Curie temperature in excess of 400°C and which is an intermetallic compound of rhombohedral or hexagonal crystal structure analogous to Th₂Zn₁₇ and Th₂Ni₁₇ respectively wherein R is one or more rare earth elements, X' is an element of groups IIIA, IIIB, IVA or IVB of the periodic table of elements, Z is one or more elements of group VA of the periodic table of elements and is interstitially incorporated into the crystal lattice of said intermetallic compound, x is a value from 0.5 to 2, y is a value from 9 to 19, a is a value from 0 to 3, b is a value from 0.3 to 3 and Fe is unsubstituted or up to 33% substituted by a transition metal with the proviso that the element X' is not boron when the component Z is antimony or bismuth.

In accordance with a second aspect the invention provides a magnetic material of the general formula

RₓFe_{y}Z_{b}

which has a Curie temperature in excess of 400°C and which is an intermetallic compound of tetragonal crystal structure analogous to ThMn₁₂ wherein R is one or more rare earth elements, Z is one or more elements of group VA of the periodic table of elements and is interstititally incorporated into the crystal lattice of said intermetallic compound, x is a value from 0.5 to 2, y is a value from 9 to 19, b is a value from 0.3 to 3 and Fe is partially substituted by an element of group IIIA or IVA of the periodic table or a transition metal from another group wherein the level of substitution of Fe with any transition metal is up to 33%.

It is to be understood that herein the term rare earth element includes the elements yttrium and thorium, and that the groups IIIA, IIIB, IVA, IVB and V of the periodic table are those defined by the CAS version of that table. By hexagonal, rhombohedral and tetragonal crystal structure is meant intermetallic compounds having a crystal structure analogous to Th₂Ni_{17'} Th₂Zn₁₇ and ThMn₁₂ respectively.

In the case where the material is an intermetallic compound of hexagonal or rhombohedral crystal structure the element R may be samarium alone or a combination of samarium with one or more other rare earth elements selected from lanthanum, cerium, neodymium, praseodymium, erbium, thulium, yttrium, and mischmetal. R may also be yttrium, cerium, neodymium, gadolinium, terbium, dysprosium, holmium, erbium, thulium, ytterbium, lutetium, or a mixture of two or more thereof. In the case where the material is an intermetallic compound of tetragonal crystal structure, R may be any rare earth element but preferred elements for R are cerium, praseodymium, neodymium, terbium, dysprosium, holmium or a mixture of two or more thereof. Particularly preferred are neodymium or praseodymium alone or in combination with other elements.

As aforementioned in the materials of the invention the iron may be substituted by up to 33% with another element or elements, in particular a transition metal, preferably a magnetic transition metal. For hexagonal or rhombohedral materials a preferred transition metal is cobalt.

In the case of the tetragonal materials as aforementioned the iron is substituted with any element of group IIIA or IVA of the periodic table or with a transition metal not already included in those groups. Preferred substituents are silicon or aluminium or any of the transition metals titanium, vandium, molydenum or chromium.

Where an element X' is included in the hexagonal or rhombohedral materials it is preferably carbon, boron, silicon or zirconium and the value of "a" may be as low as 0.1 with a maximum of 3. Preferably the value of a+b is ≦ 3.

The component Z may be nitrogen, phosphorus arsenic, antimony or bismuth or mixtures thereof and of these the particularly preferred element is nitrogen. For example, three materials in accordance with the invention which demonstrate the requisite improved magnetic properties are Sm₂Fe₁₇N_{2.3}, Sm₂Fe₁₇C_{1.1}N_{1.1} and NdFe₁₁TiN_{0.8}.

The magnetic materials of the invention display considerably improved magnetic properties over materials hitherto known. Firstly they have Curie temperatures in excess of 400°C. Secondly, they have improved easy uniaxial anisotropy as demonstrated by X-ray diffraction patterns of the material after a magnetic field has been applied. Thirdly, the magnetic moment is increased and finally the magnetic moment is subject to little variation with time or temperature around ambient temperature. These increased intrinsic magnetic properties are all very favourable for permanent magnet applications.

In accordance with a third aspect of the invention there is provided a process for modifying the magnetic properties of an intermetallic compound comprising at least one or more rare earth elements and the element iron in which the iron is optionally substituted with another element to make the compounds hereinbefore defined, which process comprises heating said intermetallic compound with a gas containing at least one group VA element Z in the substantial absence of oxygen to incorporate the said at least one element Z interstitially into the crystal lattice of the intermetallic compound by a gas-solid reaction. Where the intermetallic compound is of tetragonal crystal structure the iron may be substituted by an element of group IIIA or group IVA of the periodic table or by a transition metal not already included in those groups.

The sample material is preferably placed in a sealed container from which the oxygen can be pumped and the reactive gas added and heated from the outside. Its temperature is raised to a maximum not exceeding about 600°C. Optionally the intermetallic starting material is ground from, for example, an ingot to a particle size of from 0.5 to 50 µm diameter before heating in a suitable gas. The preferred range is 0.5 to 20 µm. Specific additives such as niobium or vanadium may be added to reduce or eliminate free iron present in the ingot faciliating the development of coercivity in the resulting modified metallic material. Alternatively, the starting material may be prepared into thin flakes or ribbons by melt spinning or into powder by mechanical alloying or spray casting. The heating may proceed for a period not exceeding 8 hours, but the exact time will depend upon the gas and the solid geometry of the starting material. The precise heating time for any starting material is therefore readily calculable.

Suitable gases to be used in the process include those which produce radicals containing single atoms of a group VA element on contact with hot surfaces such as metal or quartz or by exposure to high frequency radiation, for example gaseous hydrides of the group VA elements.

The preferred magnetic materials of the invention, in which the group VA component Z interstitially inserted into the crystal lattice is nitrogen, may be made from the appropriate intermetallic starting material using gaseous nitrogen, ammonia or hydrazine. When an intermetallic compound of the formula R₂Fe₁₇, or RFe₁₁Ti for example, is heated with nitrogen and the gas pressure monitored, a decrease in pressure occurs which begins at about 350°C and continues until the temperature reaches 650^{o}C. The initial decrease in pressure is attributed to the reaction of nitrogen with the exemplified intermetallic compound and its incorporation into the R₂Fe₁₇ or R(FeTi)₁₂ crystal lattice. That a new compound incorporating R, Fe and N has been formed is borne out by the fact that after the heating process the sample has increased weight and there is an increase in the crystal lattice parameters i.e. unit cell volume, as shown by X-ray diffraction.

The process of producing the new preferred materials may also be carried out using ammonia instead of nitrogen. In this case there is a rise in pressure starting at approximately 350°C. The rise in pressure is explained by the fact that at 350^{o}C the ammonia decomposes to nitrogen and hydrogen. The nitrogen is taken up by the intermetallic sample as evidenced by a weight gain and increased crystal lattice parameters. It appears that once the temperature exceeds about 650°C the newly formed material decomposes to alpha-Fe and nitrides of the rare earth element or elements.

In accordance with a fourth aspect of the invention the new magnetic material produced as described herein is used for fabricating permanent magnets.

A preferred process by which this may be achieved comprises milling the magnetic material with a metal such as aluminium, copper or zinc or a solder or an organic powder or resin, magnetically aligning the material by applying a magnetic field and then heating to a temperature not sufficient to decompose the material. Preferably the magnetic material is milled with zinc. This process of forming a magnet serves to increase the coercivity essential for forming magnets.

The following figures and tables give data relating to the magnetic properties of certain preferred intermetallic compounds of the invention and by way of example demonstrate the improvement in magnetic properties over known magnetic materials.

The data presented in Table 1 demonstrate that the interstitial nitride phase R₂Fe₁₇Nb, where b is about 2.6, exists across the entire rare-earth series from Ce to Lu. The unit cell volume of the crystal lattice increases by 5 to 9% on forming the nitride and the Curie temperature Tc and spontaneous magnetization 6ₛ are greatly increased. Data further indicate that substitutions exist between nitrides of different rare earths so that properties such as magnetization or anisotropy field may be optimised for particular applications having regard to the cost of the particular rare earth component.

The data again demonstrate the improvement in magnetic properties, Tc, magnetization and unit cell volume, by interstitial incorporation of nitrogen into the crystal lattice of compounds of the general formula R_{X}Fe_{y}X'ₐ.

**Table 3**

| | |
|---|---|
| The data presented in this table demonstrate the improved easy unfaxial anisotropy with, as an example, compounds where R is samarium. The value for easy uniaxial anisotropy represented by the anisotropy field Bₐ, in Tesla was obtained by aligning the rhombohedral c-axis in the direction of an applied magnetic field. From magnetization curves on oriented powders with the field applied parallel and perpendicular to the alignment direction the values for Bₐ shown in this table were obtained. | |

| Compound | Bₐ(T) |
|---|---|
| Sm₂Fe₁₇ | < 1.0 |
| Sm₂Fe₁₇N_{2.3} | >12.0 |
| Sm₂Fe₁₇C_{1.1} | 4.0 |
| Sm₂Fe₁₇C_{1.1}N_{1.0} | >8.0 |

**Table 4**

| | | |
|---|---|---|
| The data in this table presented give deduced values for iron-iron and ion-rare earth exchange interactions based on the variation in Curie temperature for the different heavy rare earths. | | |

| Compound | ⁿR-Fe(µₒ) | ⁿFe-Fe(µₒ) |
|---|---|---|
| R₂Fe₁₇ | 225 | 181 |
| R₂Fe₁₇N_{y} | 208 | 515 |

It is deduced that the iron-iron interactions are enhanced by a factor of 2.5 in the new nitride compounds while iron-rare earth interactions are only slightly decreased.

The interstitial incorporation of an element of group VA of the periodic table, for which the example is nitrogen, into selected intermetallic compounds of the formula R₂Fe₁₇ or R₂Fe₁₇X′ₐ or R(FeM)₁₂ or R₂(FeM)₁₇ where M is a substituent element as hereinbefore defined and the improved magnetic properties achieved thereby is further demonstrated by data presented in the figures in which:
Figure 1 is a thermopiezic curve for absorption of nitrogen gas by Y₂Fe₁₇ showing the drop in pressure of gas in the chamber as nitrogen is taken up by the sample. The pressure values on cooling demonstrate that the nitrogen remains absorbed by the Y₂Fe₁₇ sample;
Figure 2 shows the isothermal reaction of nitrogen with Y₂Fe₁₇ powder, having an average grain size of approximately 2 microns diameter at 400^{o}C, 450^{o}C and 500^{o}C, the value y being the number of moles of nitrogen atoms incorporated into a mole of the sample. The data indicate that the optimum temperature range for the operations of the process of the invention is between about 450^{o}C and 600^{o}C;
Figure 3 is a thermopiezic curve for absorption of ammonia gas by Y₂Fe₁₇ at an atmosphere of approximately 1 bar. The curves of heating demonstrate an increase in pressure due to uptake of nitrogen from the ammonia. There is an increase in weight after heating the sample to 550^{o}C which is attributed to nitrogen absorption.
Figure 4 shows ⁵⁷Fe Mössbauer spectra at room temperature of Y₂Fe₁₇ before (a) and after (b) heating to 500^{o}C in 1 bar ammonia. The changes in Curie temperature and magnetic moment are reflected in the ⁵⁷Fe Mossbauer spectra in which the average hyperfine field at 20^{o}C, <B_{hf}> increases from 10 Tesla for Y₂Fe₁₇ to 30 Tesla for Y₂Fe₁₇N_{2.6};
Figure 5 shows the X-ray diffraction patterns of Y₂Fe₁₇ powder heated in a thermopiezic analyser in nitrogen at 10^{o}C/minute up to the temperatures of 500^{o}C, 550^{o}C, 600^{o}C, 700^{o}C and 850^{o}C. Powders of the formula R₂Fe₁₇ where R is another rare earth element behave similarly.

The figure shows the appearance of a phase with expanded lattice parameters which co-exists with the unexpanded phase after treatment up to 550^{o}C. The Y₂Fe₁₇N_{2.6} phase forms clearly at 600^{o}C and on heating up to 700^{o}C or above the alloy decomposes to YN and αFe;
Figure 6 shows X-ray diffraction patterns of Y₂Fe₁₇ powder after heating in nitrogen gas isothermally at 500^{o}C for two hours. The extended heat treatment produces the Y₂Fe₁₇N_{2.6} compound at a lower temperature than shown in the previous figure but further heat treatment to 850^{o}C results in decomposition to YN and αFe.
Figure 7 is a thermopiezic curve for Y₂Fe₁₇C_{1.0} heated from room temperature in an atmosphere of approximately 1 bar ammonia. Again an increase in pressure at about 370^{o}C is observed;
Figure 8 shows the dependence of the Curie temperature (a) Tc(^{o}C) and the unit cell volume of the lattice (b) V(Å³) on the maximum heating temperature Tm for Y₂Fe₁₇C. For the sample treated at 450^{o}C and 500^{o}C there co-exist two R₂Fe₁₇-type phases one with the larger unit cell volume and higher Curie temperature and the other with the smaller unit cell volume and lower Curie temperature. The more the crystal lattice is expanded the higher the Curie temperature. There is also a substantial increase in spontaneous magnetic moment (µₒMₛ) to 1.46 Tesla (see Table 2);
Figure 9 shows Mossbauer spectra at room temperature of Y₂Fe₁₇C_{1.0} before (a) and after (b) heating in 1 bar ammonia at 550^{o}C. The average hyperfine field at 18^{o}C <B_{hf}> increases from 25.3 Tesla to 30.8 Tesla after the ammonia treatment;
Figure 10 is a thermopiezic curve for Sm₂Fe₁₇C_{1.1} heated from room temperature in an atmosphere of approximately 1 bar ammonia. Again an increase in pressure is shown at about 350^{o}C. Analysis of the sample after heating to 600^{o}C reveals that the material retains the rhombohedral (Th₂Zn₁₇-type) structure with increased lattice parameters. From the increase in mass the nitrogen content is estimated to be 1.1 nitrogen atoms per Sm₂Fe₁₇C_{1.1} formula unit;
Figure 11 is an X-ray diffraction pattern of Sm₂Fe₁₇C_{1.1}N_{1.1} powder before (a) and after (b) orientation in an applied field of 1.2 Tesla for one hour. The figure demonstrates the strong uniaxial anisotropy possessed in particular where R is samarium;
Figure 12 shows magnetization curves at 18^{o}C of oriented samples of Sm₂Fe₁₇C_{1.1} before (a) and after (b) treatment in 1 bar ammonia up to 600^{o}C. Curves are shown for the field applied parallel (∥) and perpendicular (⊥) to the axis of orientation. From these magnetization curves the values for µₒMₛ shown in Table 2 and Bₐ shown in Table 3 are obtained;
Figure 13 shows the X-ray diffraction patterns of a) Sm₂Fe₁₇ powder with an average particle size of 1µm and b) the same powder heated at 500^{o}C in nitrogen gas for two hours to form Sm₂Fe₁₇N_{2.4};
Figures 14a and b show the radial distribution functions deduced from extended X-ray absorption fine structure data on the same samples as Figure 13. The peak appearing at 2.5 Å shows the presence of approximately three nitrogen atoms at a distance 2.5 A from a samarium atom in the nitride;
Figures 15a and b show the crystal structure of the rhombohedral and hexagonal 2:17 structure, indicating the sites occupied by nitrogen; Figure 15a is the rhombohedral crystal structure and Figure 15b is the hexagonal crystal structure. Large circles represent rare earths, small shaded circles represent iron and small black circles represent nitrogen sites 9e or 6h.
Figure 16 is a histogram of the particle size distribution of a typical Sm₂Fe₁₇ powder used for nitrogen absorption;
Figure 17 shows the variation of the diffusion coefficient for nitrogen in the Sm₂Fe₁₇ powder as a function of inverse temperature.
Figure 18 shows magnetization curves at 18°C for an oriented sample of Sm₂Fe₁₇N_{2.3} after treatment with ammonia. Again curves are shown for the field applied parallel (∥) and perpendicular (⊥) to the axis of orientation. From these the values of the anisotropy field Bₐ are obtained as shown in Table 3. The value of Bₐ for Sm₂Fe₁₇N_{2.3} is given as >12.0 Tesla but in fact the curves shown in the figure indicate it may be as high as 20 Tesla;
Figure 19(a) is a thermopiezic curve for a powder made from a cast ingot of Sm₂Fe₁₇ heated in nitrogen. Figure 19(b) is a thermopiezic curve for a powder made from an ingot and annealed for 100 hours at 950^{o}C and heated in nitrogen. The differences in the two sets of curves clearly demonstrate that the treatment temperature required to form the R₂Fe₁₇N_{b} phase varies depending on the metallurgical composition of the ingot used to make the powder;
Figure 20 shows X-ray diffraction patterns of the compounds Nd₂Fe₁₇N_{2.3}, Sm₂Fe₁₇N_{2.3} and Er₂Fe₁₇N_{2.7} after an applied field of 1.2 Tesla. In the case of Sm₂Fe₁₇N_{2.3} the c-axis is aligned parallel to the applied field indicating strong uniaxial anisotropy. However in the case where R is Nd or Er there is a tendency for the c-axis to be aligned perpendicular to the direction of the applied magnetic field;
Figure 21 shows the crystal structure of the tetragonal 1:12 compound showing sites occupied by nitrogen. The coding of the circles is as described for Figures 15a and 15b;
Figure 22 shows a thermopiezic trace for absorption of nitrogen gas by Sm(Fe₁₁Ti). The material was heated at a rate of 10^{o}C/minute at approximately 1 bar nitrogen. The figure demonstrates that the optimum temperature range for operation of the process is similar to that of the R₂Fe₁₇ compounds;
Figure 23 shows room temperature ⁵⁷ Mössbauer spectra of Sm(Fe₁₁Ti) before (a) and after (b) heating in a nitrogen containing gas in accordance with the invention. The average hypefine field increases from 25.5 Tesla in (a) to 29.1 Tesla in (b), reflecting the changes in Curie temperature and iron magnetic moment.
Figure 24 shows X-ray diffraction patterns of powders of Sm(Fe₁₁Ti) (a) and Sm(Fe₁₁Ti)N_{0.8} (b) oriented in a magnetic field of 1.2 Tesla. The strong uniaxial anisotropy of Sm(Fe₁₁Ti) is transformed to easy-plane anisotropy in the interstitial nitride SmFe₁₁TiN_{0.8} demonstrating a change in sign of the second-order crystal field coefficient A₂₀ from negative to positive. Hence the strong uniaxial anisotropy observed for interstitially-modified 1:12 structure compounds of rare-earths with a negative Stevens coefficient α_{J}(Nd,Er,Tm), neodymium in particular;
Figure 25 is an illustration of interstitial nitrogen atoms around the rare earth in the rhombohedral or hexagonal 2.17 structure (a) and in the tetragonal 1.12 structure (b). The electric field gradient experienced by the rare-earth, quantified in the parameter A₂₀, is mainly produced by surrounding interstitial atoms in the materials of the invention. It is negative for the configuration of the 2.17 compounds and positive for configuration of the 1.12 compounds;
Figure 26 illustrates some of the effects of cobalt substitution for iron in materials of the invention having the rhombohedral or hexagonal crystal structure.
Figure 26(a) indicates the nitrogen content achieved by treating finely-ground powders of the R₂(Fe_{17-c}Co_{c})N_{b} type formula where c is the number of cobalt atoms in nitrogen gas at temperatures ranging from 400-600^{o}C.
Figure 26(b) illustrates a broad maximum in magnetization with a transition metal substitute where R is Y and c=0.2.
Figure 26(c) shows that the transition metal substituents make a positive contribution to the anisotropy when c is >0.1;
Figure 27 is an illustration of the development of hysteresis in a powder of Sm₂Fe₁₇N_{2.3} comprising first and second quadrant demagnetizing curves of samples aligned and magnetized in a pulsed field of 8 Tesla. The data represented are as follows:
   a) Powder of Sm₂Fe₁₇N_{2.3} dispersed in epoxy resin
   b) Powder of Sm₂Fe₁₇N_{2.3} milled with Zn powder (25 wt %)
   c) Powder of Sm₂Fe₁₇N_{2.3} milled with Zn powder (15 wt %) and heat treated at 400^{o}C for two hours.
Figure 27 indicates the magnetic properties of permanent magnets produced from the magnetic materials of the invention and methods by which the coercivity and hysteresis may be developed. For example in 21(c) the material is milled with 15 wt % Zn and heated to 400^{o}C to produce a magnet having a coercivity of 0.5 Tesla and a maximum energy product of 86KJm⁻³.

The data shown in Figure 27 establishes conclusively that Sm₂Fe₁₇N_{2.3} and the related compounds of the invention can be effectively processed to make magnets.

Further, thin films of materials of the invention may be exploited for magnetic or magneto-optic recording.

## Claims (Claims for the following Contracting State(s): DE, GB, FR, IT, HL, SE, CH, LI, BE, AT, LU, GR, DK)

1. A magnetic material of the general formula:
RₓFe_{y}X'ₐZ_{b}
which has a Curie temperature in excess of 400°C and which is an intermetallic compound of rhombohedral or hexagonal crystal structure analogous to Th₂Zn₁₇ and Th₂Ni₁₇ respectively wherein R is one or more rare earth elements, X' is an element of groups IIIA, IIIB, IVA or IVB of the periodic table of elements, Z is one or more elements of group VA of the periodic table of elements and is interstitially incorporated into the crystal lattice of said intermetallic compound, x is a value from 0.5 to 2, y is a value from 9 to 19, a is a value from 0 to 3, b is a value from 0.3 to 3 and Fe is unsubstituted or up to 33% substituted by a transition metal with the proviso that the element X' is not boron when the component Z is antimony or bismuth.

2. A magnetic material of the general formula:
RₓFe_{y}Z_{b}
which has a Curie temperature in excess of 400°C and which is an intermetallic compound of tetragonal crystal structure analogous to ThMn₁₂ wherein R is one or more rare earth elements, Z is one or more elements of group VA of the periodic table of elements and is interstititally incorporated into the crystal lattice of said intermetallic compound, x is a value from 0.5 to 2, y is a value from 9 to 19, b is a value from 0.3 to 3 and Fe is partially substituted by an element of group IIIA or IVA of the periodic table or a transition metal from another group wherein the level of substitution of Fe with any transition metal is up to 33%.

3. A magnetic material as claimed in claim 1 or 2 wherein R is samarium or neodymium.

4. A magnetic material as claimed in claim 1 or claim 3 wherein R is samarium.

5. A magnetic material as claimed in claim 1 wherein R is samarium in combination with one or more rare earth elements selected from yttrium, lanthanum, cerium, neodymium, erbium, thulium and mischmetal.

6. A magnetic material as claimed in claim 1 wherein R is yttrium, lanthanum, cerium, praseodymium, neodymium, gadolinium, terbium, dysprosium, erbium, thulium, ytterbium or lutetium or a mixture of two or more thereof.

7. A magnetic material as claimed in claim 2 wherein R is yttrium, thorium, cerium, praseodymium, neodymium, terbium, dysprosium or holmium or a mixture of two or more thereof.

8. A magnetic material as claimed in any preceding claim wherein the transition metal is cobalt.

9. A magnetic material as claimed in any one of claims 2, 3 or 7 wherein the iron is partially substituted by titanium, vanadium, molybdenum or chromium.

10. A magnetic material as claimed in any one of claims 2,3 or 7 wherein the iron is partially substituted by aluminium or silicon.

11. A magnetic material as claimed in any of claims 1,3,4,5 or 6 wherein X' is carbon, boron, silicon or zirconium and a is a value from 0.1 to 3.

12. A magnetic material as claimed in claim 11 wherein a+b ≦ 3.

13. A magnetic material as claimed in any preceding claim wherein Z is nitrogen.

14. A magnetic material as claimed in any one of claims 1 to 12 wherein Z is a combination of nitrogen with one or more other group VA elements.

15. A magnetic material as claimed in any one of claims 1 to 12 wherein component Z is one or more of P, As, Sb and Bi.

16. A magnetic material as claimed in claim 13 which has the formula sm₂Fe₁₇N_{2.3} or Sm₂Fe₁₇C_{1.1}N_{1.1} or NdFe₁₁TiN_{0.8}.

17. A process for modifying the magnetic properties of an intermetallic compound comprising at least one or more rare earth elements and the element iron to produce a magnetic material as defined in any one of claims 1 to 16 which process comprises heating said intermetallic compound with a gas containing at least one group VA element Z in the substantial absence of oxygen to incorporate the said at least one element Z interstitially into the crystal lattice of the intermetallic compound by a gas-solid reaction.

18. A process as claimed in claim 17 wherein the gas is one which produces radicals containing single atoms of the group VA element Z on contact with hot surfaces such as metal or quartz or by exposure to high frequency radiation.

19. A process as claimed in claim 18 wherein the gas is a gaseous hydride of the group VA element Z.

20. A process as claimed in claim 18 wherein the group VA element Z is nitrogen and the gas is nitrogen, ammonia or hydrazine.

21. A process as claimed in any one of claims 17 to 20 wherein said intermetallic compound is heated to a temperature not exceeding 650°C.

22. A process as claimed in any one of claims 17 to 21 wherein said intermetallic compound is ground to a particle size of 1 to 50 µm diameter.

23. A process as claimed in claim 22 wherein the said ground compound is heated for up to 8 hours.

24. Use of the magnetic material as claimed in any one of claims 1 to 16 for fabricating a permanent magnet.

25. A process of fabricating a permanent magnet from a magnetic material as claimed in any one of claims 1 to 16 by a process comprising the steps of:-
a) milling said magnetic material with a metal such as aluminium, copper or zinc or an organic powder or resin
b) generating magnetic alignment in the said material by applying a magnetic field and
c) heating the milled product to a temperature sufficiently low to prevent decomposition of the magnetic material.

26. A method as claimed in claim 25 wherein in the magnet fabricating process the magnetic material is milled with from 5 to 20 wt % zinc.

27. A permanent magnet comprising a magnetic material as claimed in any one or claims 1 to 16.

28. A permanent magnet comprising a magnetic material which is produced by the process of any one of claims 17 to 23.

## Claims (Claims for the following Contracting State(s): ES)

1. A process for modifying the magnetic properties of an intermetallic compound comprising at least one or more rare earth elements and the element iron to produce a magnetic material of the general formula:-
RₓFe_{y}X'ₐZ_{b}
which has a Curie temperature in excess of 400°C and which is an intermetallic compound of rhombohedral or hexagonal crystal structure analogous to Th₂Zn₁₇ and Th₂Ni₁₇ respectively wherein R is one or more rare earth elements, X' is an element of groups IIIA, IIIB, IVA or IVB of the periodic table of elements, Z is one or more elements of group VA of the periodic table of elements and is interstitially incorporated into the crystal lattice of said intermetallic compound, x is a value from 0.5 to 2, y is a value from 9 to 19, a is a value from 0 to 3, b is a value from 0.3 to 3 and Fe is unsubstituted or up to 33% substituted by a transition metal with the proviso that the element X' is not boron when the component Z is antimony or bismuth; which process comprises heating said intermetallic compound in a gas containing Z in the substantial absence of oxygen to incorporate Z interstitially into the crystal lattice of the intermetallic compound by a gas-solid reaction.

2. A process for modifying the magnetic properties of an intermetallic compound comprising at least one or more rare earth elements and the element iron to produce a magnetic material of the general formula:-
RₓFe_{y}Z_{b}
which has a Curie temperature in excess of 400°C and which is an intermetallic compound of tetragonal crystal structure analogous to ThMn₁₂ wherein R is one or more rare earth elements, Z is one or more elements of group VA of the periodic table of elements and is interstititally incorporated into the crystal lattice of said intermetallic compound, x is a value from 0.5 to 2, y is a value from 9 to 19, b is a value from 0.3 to 3 and Fe is partially substituted by an element of group IIIA or IVA of the periodic table or a transition metal from another group wherein the level of substitution of Fe with any transition metal is up to 33%; which process comprises heating, said intermetallic compound in a gas containing Z in the substantial absence of oxygen to incorporate Z interstitially into the crystal lattice of the intermetallic compound by a gas solid reaction.

3. A process as claimed in claim 1 or claim 2 wherein the gas is one which produces radicals containing single atoms of the group VA element Z on contact with hot surfaces such as metal or quartz or by exposure to high frequency radiation.

4. A process as claimed in claim 3 wherein the gas is a gaseous hydride of the group VA element Z.

5. A process as claimed in claim 3 wherein the group VA element Z is nitrogen and the gas is nitrogen, ammonia or hydrazine.

6. A process as claimed in any one of claims 1 to 5 wherein said intermetallic compound is heated to a temperature not exceeding 650°C.

7. A process as claimed in any one of claims 1 to 6 wherein said intermetallic compound is ground to a particle size of 1 to 50 µm diameter.

8. A process as claimed in claim 7 wherein the said ground compound is heated for up to 8 hours.

9. A process as claimed in any preceding claim wherein R is samarium or neodynium.

10. A process as claimed in any one of claims 1 and 3 to 8 wherein R is samarium.

11. A process as claimed in any one of claims 1 and 3 to 8 wherein R is samarium in combination with one or more rare earth elements selected from yttrium, lanthanum, cerium, neodymium, erbium, thulium and mischmetal.

12. A process as claimed in any one of claims 1 and 3 to 8 wherein R is yttrium, lanthanum, cerium, praseodymium, neodymium, gadolinium, terbium, dysprosium, erbium, thulium, ytterbium or lutetium or a mixture of two or more thereof.

13. A process as claimed in any one of claims 2 to 8 wherein R is yttrium, thorium, cerium, praseodymium, neodymium, terbium, dysprosium or holmium or a mixture of two or more thereof.

14. A process as claimed in claim 1 or any of claims 3 to 12 wherein the transition metal is cobalt.

15. A process as claimed in any one of claims 2 to 8 and 13 wherein the element Fe is partially substituted by titanium, vanadium, molydenum or chromium.

16. A process as claimed in any one of claims 2 to 8 and 13 wherein the element Fe is partially substituted by aluminium or silicon.

17. A process as claimed in any of claims 1 and 3 to 12 wherein X' is carbon, boron, silicon or zirconium and a is a value from 0.1 to 3.

18. A process as claimed in claim 16 wherein a+b ≦ 3.

19. A process as claimed in any preceding claim wherein Z is nitrogen.

20. A process as claimed in any one of claims 1 to 18 wherein Z is a combination of nitrogen with one or more other group VA elements.

21. A process as claimed in any one of claims 1 to 18 wherein Z is one or more of P, As, Sb and Bi.

22. Use of the magnetic material made by the process as claimed in any preceding claim for fabricating a permanent magnet.

23. A method of fabricating a permanent magnet from a magnetic material made by the process of any of claims 1 to 21 comprising the steps of:
a) milling said magnetic material with a metal such as aluminium, copper or zinc or an organic powder or resin
b) generating magnetic alignment in the said material by applying a magnetic field and
c) heating the milled product to a temperature sufficiently low to prevent decomposition of the magnetic material.

24. A method as claimed in claim 23 wherein in the magnet fabricating process the magnetic material is milled with from 5 to 20 wt % zinc.

25. A permanent magnet comprising a magnetic material which is produced by the process as claimed in any one of claims 1 to 21.

## Patentansprüche (Patentansprüche für folgende(n) Vertragsstaat(en): DE, GB, FR, IT, NL, SE, CH, LI, BE, AT, LU, GR, DK)

1. Magnetisches Material des allgemeinen Formel :
RₓFe_{y}X'ₐZ_{b'}
mit einer Curie-Temperatur von über 400°C und, welches eine zu Th₂Zn₁₇ bzw. Th₂Ni₁₇ analoge intermetallische Verbindung mit rhomboedrischer oder hexagonaler Kristallstruktur ist, worin R eines oder mehrere Seltenerdelemente ist, X' ein Element der Gruppen IIIA, IIIB, IVA oder IVB des perodischen Systems der Elemente ist, Z eines oder mehrere der Elemente der Gruppe VA des Periodensystems der Elemente ist und interstitiell in das Kristallgitter der intermetallischen Verbindung eingelagert ist, x ein Wert von 0,5 bis 2 ist, y ein Wert von 9 bis 19 ist, a ein Wert von 0 bis 3 ist, b ein Wert von 0,3 bis 3 ist und Eisen unsubstituiert oder bis zu 33 % durch ein Übergangsmetall substituiert ist, mit der Maßgabe daß das Element X' nicht Bor ist, wenn die komponente Z Antimon oder Bismut ist.

2. Magnetisches Material der allgemeinen Formel:
RₓFe_{y}Z_{b'}
mit einer Curie-Temperatur von über 400°C und welches eine zu ThMn₁₂ analoge intermetallische Verbindung mit tetragonaler Kristallstruktur ist, worin R eines oder mehrere Seltenerdelemente ist, Z eines oder mehrere der Elemente der Gruppe VA des Periodensystems der Elemente ist und interstitiell in das Kristallgitter der intermetallischen Verbindung eingelagert ist, x ein Wert von 0,5 bis 2 ist, y ein Wert von 9 bis 19 ist, b ein Wert von 0,3 bis 3 ist und Eisen partiell durch ein Element der Gruppe IIIA oder IVA des Periodensystems oder durch ein Übergangsmetall aus einer anderen Gruppe substituiert ist, worin der Substitutionsgrad von Fe durch ein Übergangsmetall bis zu 33 % ist.

3. Magnetisches Material nach Anspruch 1 oder 2, worin R Samarium oder Neodymium ist.

4. Magnetisches Material nach Anspruch 1 oder 3, worin R Samarium ist.

5. Magnetisches Material nach Anspruch 1, worin R Samarium in Kombination mit einem oder mehreren Seltenerdelementen, ausgewählt aus Yttrium, Lanthan, Cerium, Neodymium, Erbium, Thulium und Mischmetall, ist.

6. Magnetisches Material nach Anspruch 1, worin R Yttrium, Lanthan, Cerium, Praseodymium, Neodymium, Gadolinium, Terbium, Dysprosium, Erbium, Thulium, Ytterbium oder Lutetium oder ein Gemisch von zwei oder mehreren davon ist.

7. Magnetisches Material nach Anspruch 2, worin R Yttrium, Thorium, Cerium, Praseodymium, Neodymium, Terbium, Dysprosium oder Holmium oder ein Gemisch von zwei oder mehreren davon ist.

8. Magnetisches Material nach einem der vorhergehenden Ansprüche, worin das Übergangsmetall Kobalt ist.

9. Magnetisches Material nach einem der Ansprüche 2, 3 oder 7, worin Eisen teilweise durch Titan, Vanadium, Molybdän oder Chrom teiweise substituiert ist.

10. Magnetisches Material nach einem der Ansprüche 2, 3 oder 7, worin Eisen teilweise durch Aluminium oder Silicium substituiert ist.

11. Magnetisches Material nach einem der Ansprüche 1, 3, 4, 5 oder 6, worin X' Kohlenstoff, Bor, Silicium oder Zirkonium ist und a ein Wert von 0,1 bis 3 ist.

12. Magnetisches Material nach Anspruch 11, worin a+b ≤ 3 ist.

13. Magnetisches Material nach einem der vorhergehenden Ansprüche, worin Z Stickstoff ist.

14. Magnetisches Material nach einem der Ansprüche 1 bis 12, worin Z eine Kombination von Stickstoff mit einem oder mehreren anderen Gruppe VA-Elementen ist.

15. Magnetisches Material nach einem der Ansprüche 1 bis 12, worin die Komponente Z eines oder mehrere aus P, As, Sb oder Bi ist.

16. Magnetisches Material nach Anspruch 13, mit der Formel Sm₂Fe₁₇N_{2,3} oder Sm₂Fe₁₇C_{1,1}N_{1,1} oder NdFe₁₁TiN_{0,8}.

17. Verfahren zum Modifizieren der magnetischen Eigenschaften einer intermetallischen Verbindung, umfassend mindestens eines oder mehrere Seltenerdelemente und das Element Eisen, um ein magnetisches Material nach einem der Ansprüche 1 bis 16 herzustellen, wobei das Verfahren das Erhitzen der intermetallischen Verbindung mit einem Gas, das mindestens ein Gruppe VA-Element Z enthält, im wesentlichen unter Abwesenheit von Sauerstoff, umfaBt, um mindestens ein Element Z interstitiell in das Kristallgitter der intermetallischen Verbindung durch eine Gas-Feststoff-Reaktion einzubringen.

18. Verfahren nach Anspruch 17, worin das Gas ein derartiges ist, welches beim Kontakt mit heißen Oberflächen, wie etwa Metall oder Quarz, oder durch Behandeln mit Hochfrequenzstrahlung Reste erzeugt, die einzelne Atome des Gruppe-VA-Elements Z enthalten.

19. Verfahren nach Anspruch 18, worin das Gas ein gasförmiges Hydrid des Gruppe VA-Elements Z ist.

20. Verfahren nach Anspruch 18, worin das Gruppe VA-Element Z Stickstoff ist und das Gas Stickstoff, Ammoniak oder Hydrazin ist.

21. Verfahren nach einem der Ansprüche 17 bis 20, worin die intermetallische Verbindung auf eine Temperatur von nicht über 650°C erhitzt wird.

22. Verfahren nach einem der Ansprüche 17 bis 21, worin die intermetallische Verbindung auf eine Teilchengröße von 1 bis 50 µm Durchmesser gemahlen wird.

23. Verfahren nach Anspruch 22, worin die gemahlene Verbindung für bis zu 8 Stunden erhitzt wird.

24. Verwendung des magnetischen Materials nach einem der Ansprüche 1 bis 16 zum Herstellen eines Permanentmagneten.

25. Verfahren zum Herstellen eines Permanentmagneten aus einem magnetischen Material nach einem der Ansprüche 1 bis 16 durch ein Verfahren, umfassend die Schritte:
a) Mahlen des magnetischen Materials mit einem Metall, wie etwa Aluminium, Kupfer oder Zink oder einem organischen Pulver oder Harz,
b) Erzeugen einer magnetischen Ausrichtung in dem Material durch Anlegen eines magnetischen Feldes, und
c) Erhitzen des gemahlenen Produkts auf eine Temperatur, die ausreichend niedrig ist, um eine Zersetzung des magnetischen Materials zu verhindern.

26. Verfahren nach Anspruch 25, worin in dem Magnetherstellungsverfahren das magnetische Material mit von 5 bis 20 Gew.-% Zink gemahlen wird.

27. Permanentmagnet, umfassend ein magnetisches Material nach einem der Ansprüche 1 bis 16.

28. Permanentmagnet, umfassend ein magnetisches Material, das durch das Verfahren nach einen der Ansprüche 17 bis 23 hergestellt wurde.

## Patentansprüche (Patentansprüche für folgende(n) Vertragsstaat(en): ES)

1. Verfahren zum Modifizieren der magnetischen Eigenschaften einer intermetallischen Verbindung, umfassend mindestens eines oder mehrere Seltenerdelemente und das Element Eisen, um ein magnetisches Material der allgemeinen Formel:
RₓFe_{y}X'ₐZ_{b}
herzustellen, welches eine Curie-Temperatur von über 400°C hat und welches, eine zu Th₂Zn₁₇ bzw. Th₂Ni₁₇ analoge intermetallische Verbindung mit rhomboedrischer oder hexagonaler Kristallstruktur ist, worin R eines oder mehrere Seltenerdelemente ist, X' ein Element der Gruppen IIIA, IIIB, IVA oder IVB des Periodensystems der Elemente ist, Z eines oder mehrere der Elemente der Gruppe VA des Periodensystems der Elemente ist und interstitiell in das Kristallgitter der intermetallischen Verbindung eingelagert ist, x ein Wert von 0,5 bis 2 ist, y ein Wert von 9 bis 19 ist, a ein Wert von 0 bis 3 ist, b ein Wert von 0,3 bis 3 ist und Eisen unsubstituiert oder bis zu 33 % durch ein Übergangsmetall substituiert ist, mit der Maßgabe, daß das Element X' nicht Bor ist, wenn die Komponente Z Antimon oder Bismut ist, wobei das Verfahren das Erhitzen der intermetallischen Verbindung in einem Gas, das Z enthält, im wesentlichen unter Abwesenheit von Sauerstoff, umfaßt, um Z interstitiell in das Kristallgitter der intermetallischen Verbindung durch eine Gas-Feststoff-Reaktion einzubringen.

2. Verfahren zum modifizieren der magnetischen Eigenschaften einer interstitiellen Verbindung, umfassend mindestens eines oder mehrere Seltenerdelemente und das Element Eisen, um ein magnetisches Material der allgemeinen Formel:
RₓFe_{y}Z_{b}
zu bilden, welches eine Curie-Temperatur von über 400°C hat und welches eine zu ThMn₁₂ analoge intermetallische Verbindung mit tetragonaler Kristallstruktur ist, worin R eines oder mehrere Seltenerdelemente ist, Z eines oder mehrere der Elemente der Gruppe VA des Periodensystems ist und interstitiell in das Kristallgitter der intermetallischen Verbindung eingelagert ist, x ein Wert von 0,5 bis 2 ist, y ein Wert von 9 bis 19 ist, b ein Wert von 0,3 bis 3 ist und Eisen partiell durch ein Element der Gruppe IIIA oder IVA des Periodensystems oder durch ein Übergangsmetall aus einer anderen Gruppe substituiert ist, worin der Substitutionsgrad von Fe durch ein Übergangsmetall bis zu 33 % ist, wobei das Verfahren das Erhitzen der intermetallischen Verbindung in einem Gas, das Z enthält, im wesentlichen unter Abwesenheit von Sauerstoff, umfaßt, um Z interstitiell in das Kristallgitter der intermetallischen Verbindung durch eine Gas-Feststoff-Reaktion einzubringen.

3. Verfahren nach Anspruch 1 oder 2, worin das Gas ein derartiges ist, welches beim Kontakt mit heißen Oberflächen, wie etwa Metall oder Quarz, oder durch Behandeln mit Hochfrequenzstrahlung Reste erzeugt, die einzelne Atome des Gruppe-VA-Elements Z enthalten.

4. Verfahren nach Anspruch 3, worin das Gas ein gasförmiges Hydrid des Gruppe VA-Elements Z ist.

5. Verfahren nach Anspruch 3, worin das Gruppe VA-Element Z Stickstoff ist und das Gas Stickstoff, Ammoniak oder Hydrazin ist.

6. Verfahren nach einem der Ansprüche 1 bis 5, worin die intermetallische Verbindung auf eine Temperatur von nicht über 650°C erhitzt wird.

7. Verfahren nach einem der Ansprüche 1 bis 6, worin die intermetallische Verbindung auf eine Teilchengröße von 1 bis 50 µm Durchmesser gemahlen wird.

8. Verfahren nach Anspruch 7, worin die gemahlene Verbindung für bis zu 8 Stunden erhitzt wird.

9. Verfahren nach einem der vorhergehenden Ansprüche, worin R Samarium oder Neodymium ist.

10. Verfahren nach einem der Ansprüche 1 und 3 bis 8, worin R Samarium ist.

11. Verfahren nach einem der Ansprüche 1 und 3 bis 8, worin R Samarium in Kombination mit einem oder mehreren Seltenerdelementen, ausgewählt aus Yttrium, Lanthan, Cerium, Neodymium, Erbium, Thulium und Mischmetall, ist.

12. Verfahren nach einem der Ansprüche 1 und 3 bis 8, worin R Yttrium, Lanthan, Cerium, Praseodymium, Neodymium, Gadolinium, Terbium, Dysprosium, Erbium, Thulium, Ytterbium oder Lutetium oder ein Gemisch von zwei oder mehreren davon ist.

13. Verfahren nach einem der Ansprüche 2 bis 8, worin R Yttrium, Thorium, Cerium, Praseodymium, Neodymium, Terbium, Dysprosium oder Holmium oder ein Gemisch von zwei oder mehreren davon ist.

14. Verfahren nach Anspruch 1 oder einem der Ansprüche 3 bis 12, worin das Übergangsmetall Kobalt ist.

15. Verfahren nach einem der Ansprüche 2 bis 8 und 13, worin das Element Fe teilweise durch Titan, Vanadium, Molybdän oder Chrom substituiert ist.

16. Verfahren nach einem der Ansprüche 2 bis 8 und 13, worin das Element Fe teilweise durch Aluminium oder Silicium substituiert ist.

17. Verfahren nach einem der Ansprüche 1 und 3 bis 12, worin X' Kohlenstoff, Bor, Silicium oder Zirkonium ist und a ein Wert von 0,1 bis 3 ist.

18. Verfahren nach Anspruch 16, worin a+b ≤ 3 ist.

19. Verfahren nach einem der vorhergehenden Ansprüche, worin Z Stickstoff ist.

20. Verfahren nach einem der Ansprüche 1 bis 18, worin Z eine Kombination von Stickstoff mit einem oder mehreren anderen Gruppe VA-Elementen ist.

21. Verfahren nach einem der Ansprüche 1 bis 18, worin die Komponente Z eines oder mehrere aus P, As, Sb oder Bi ist.

22. Verwendung des magnetischen Materials, das nach einem der vorhergehenden Ansprüche hergestellt wurde, zum Herstellen eines Permanentmagneten.

23. Verfahren zum Herstellen eines Permanentmagneten aus einem magnetischen Material nach einem der Ansprüche 1 bis 21, durch ein Verfahren, umfassend die Schritte:
a) Mahlen des magnetischen Materials mit einem Metall, wie etwa Aluminium, Kupfer oder Zink oder einem organischen Pulver oder Harz,
b) Erzeugen einer magnetischen Ausrichtung in dem Material durch Anlegen eines magnetischen Feldes, und
c) Erhitzen des gemahlenen Produkts auf eine Temperatur, die ausreichend niedrig ist, um die Zersetzung des magnetischen Materials zu verhindern.

24. Verfahren nach Anspruch 23, worin in dem Magnetherstellungsverfahren das magnetische Material mit von 5 bis 20 Gew.-% Zink gemahlen wird.

25. Permanentmagnet, umfassend ein magnetisches Material, das nach einem der Ansprüche 1 bis 21 hergestellt wurde.

## Revendications (Revendications pour l'(les) Etat(s) contractant(s) suivant(s): DE, GB, FR, IT, NL, SE, CH, LI, BE, AT, LU, GR, DK)

1. Matériau magnétique répondant à la formule générale :
RₓFe_{y}X'ₐZ_{b}
ayant un point de Curie supérieur à 400°C et qui est un composé intermétallique de structure cristalline rhomboédrique ou hexagonale respectivement analogue à Th₂Zn₁₇ et Th₂Ni₁₇, où R représente un ou plusieurs éléments des terres rares, X' est un élément des groupes IIIA, IIIB, IVA ou IVB du tableau périodique des éléments, Z représente un ou plusieurs éléments du groupe VA du tableau périodique des éléments et est incorporé dans les interstices du réseau cristallin dudit composé intermétallique, x est une valeur de 0,5 à 2, y est une valeur de 9 à 19, a est une valeur de 0 à 3, b est une valeur de 0,3 à 3, et Fe est non substitué ou substitué jusqu'à 33 % par un métal de transition, avec la condition que l'élément X' ne soit pas le bore quand le composant Z est l'antimoine ou le bismuth.

2. Matériau magnétique répondant à la formule générale :
RₓFe_{y}Z_{b}
ayant un point de Curie supérieur à 400°C et qui est un composé intermétallique de structure cristalline tétragonale analogue à ThMn₁₂, où R représente un ou plusieurs éléments des terres rares, Z représente un ou plusieurs éléments du groupe VA du tableau périodique des éléments et est incorporé dans les interstices du réseau cristallin dudit composé intermétallique, x est une valeur de 0,5 à 2, y est une valeur de 9 à 19, b est une valeur de 0,3 à 3, et Fe est partiellement substitué par un élément du groupe IIIA ou IVA du tableau périodique des éléments ou par un métal de transition provenant d'un autre groupe, le taux de substitution de Fe par n'importe quel métal de transition valant jusqu'à 33 %.

3. Matériau magnétique tel que revendiqué dans la revendication 1 ou 2, où R est le samarium ou le néodyme.

4. Matériau magnétique tel que revendiqué dans la revendication 1 ou 3, où R est le samarium.

5. Matériau magnétique tel que revendiqué dans la revendication 1, où R est le samarium combiné avec un ou plusieurs éléments des terres rares, choisis parmi l'yttrium, le lanthane, le cérium, le néodyme, l'erbium, le thulium et le mischmétal.

6. Matériau magnétique tel que revendiqué dans la revendication 1, où R est l'yttrium, le lanthane, le cérium, le praséodyme, le néodyme, le gadolinium, le terbium, le dysprosium, l'erbium, le thulium, l'ytterbium ou le lutétium, ou un mélange d'au moins deux de ces éléments.

7. Matériau magnétique tel que revendiqué dans la revendication 2, où R est l'yttrium, le thorium, le cérium, le praséodyme, le néodyme, le terbium, le dysprodium ou l'holmium, ou un mélange d'au moins deux de ces éléments.

8. Matériau magnétique tel que revendiqué dans l'une quelconque des revendications précédentes, où le métal de transition est le cobalt.

9. Matériau magnétique tel que revendiqué dans l'une quelconque des revendications 2, 3 ou 7, où le fer est partiellement substitué par du titane, du vanadium, du molybdène ou du chrome.

10. Matériau magnétique tel que revendiqué dans l'une quelconque des revendications 2, 3 ou 7, où le fer est partiellement substitué par de l'aluminium ou du silicium.

11. Matériau magnétique tel que revendiqué dans l'une quelconque des revendications 1, 3, 4, 5 ou 6, où X' est le carbone, le bore, le silicium ou le zirconium, et a est une valeur de 0,1 à 3.

12. Matériau magnétique tel que revendiqué dans la revendication 11, où a+b ≤ 3.

13. Matériau magnétique tel que revendiqué dans l'une quelconque des revendications précédentes, où Z est l'azote.

14. Matériau magnétique tel que revendiqué dans l'une quelconque des revendications 1 à 12, où Z est une combinaison de l'azote avec un ou plusieurs autres éléments du groupe VA.

15. Matériau magnétique tel que revendiqué dans l'une quelconque des revendications 1 à 12, où le composant Z représente un ou plusieurs éléments choisis parmi P, As, Sb et Bi.

16. Matériau magnétique tel que revendiqué dans la revendication 13, répondant à la formule Sm₂Fe₁₇N_{2,3} ou Sm₂Fe₁₇C_{1,1} N_{1,1} ou NdFe₁₁TiN_{0,8}.

17. Procédé pour modifier les propriétés magnétiques d'un composé intermétallique comprenant au moins un ou plusieurs éléments des terres rares et l'élément fer pour produire un matériau magnétique tel que défini dans l'une quelconque des revendications 1 à 16, ledit procédé comprenant le chauffage dudit composé intermétallique avec un gaz contenant au moins un élément Z provenant du groupe VA, essentiellement en l'absence d'oxygène, pour incorporer ledit élément minimal Z dans les interstices du réseau cristallin du composé intermétallique au moyen d'une réaction du type gaz-solide.

18. Procédé tel que revendiqué dans la revendication 17, dans lequel le gaz est un gaz qui produit des radicaux contenant des atomes individuels de l'élément Z du groupe VA par contact avec des surfaces chaudes tel qu'un métal ou le quartz ou par exposition à un rayonnement à haute fréquence.

19. Procédé tel que revendiqué dans la revendication 18, dans lequel le gaz est un hydrure gazeux de l'élément Z du groupe VA.

20. Procédé tel que revendiqué dans la revendication 18, dans lequel l'élément Z du groupe VA est l'azote, et le gaz est l'azote, l'ammoniac ou l'hydrazine.

21. Procédé tel que revendiqué dans l'une quelconque des revendications 17 à 20, dans lequel ledit composé intermétallique est chauffé à une température ne dépassant pas 650°C.

22. Procédé tel que revendiqué dans l'une quelconque des revendications 17 à 21, dans lequel ledit composé intermétallique est broyé jusqu'à l'obtention d'une dimension de particules de 1 à 50 µm de diamètre.

23. Procédé tel que revendiqué dans la revendication 22, dans lequel ledit composé broyé est chauffé pendant une durée allant jusqu'à 8 heures.

24. Utilisation du matériau magnétique tel que revendiqué dans l'une quelconque des revendications 1 à 16 pour la fabrication d'un aimant permament.

25. Procédé de fabrication d'un aimant permanent à partir d'un matériau magnétique tel que revendiqué dans l'une quelconque des revendications 1 à 16, au moyen d'un procédé comprenant les étapes consistant à :
a) broyer ledit matériau magnétique avec un métal tel que l'aluminium, le cuivre ou le zinc ou une poudre organique ou une résine,
b) créer un alignement magnétique dans ledit matériau en appliquant un champ magnétique, et
c) chauffer le produit broyé à une température suffisamment basse pour empêcher la décomposition du matériau magnétique.

26. Procédé tel que revendiqué dans la revendication 25, où, dans le procédé de fabrication de l'aimant, le matériau magnétique est broyé avec 5 à 20 % en poids de zinc.

27. Aimant permanent comprenant un matériau magnétique tel que revendiqué dans l'une quelconque des revendications 1 à 16.

28. Aimant permanent comprenant un matériau magnétique qui est produit au moyen du procédé selon l'une quelconque des revendications 17 à 23.

## Revendications (Revendications pour l'(les) Etat(s) contractant(s) suivant(s): ES)

1. Procédé pour modifier les propriétés magnétiques d'un composé intermétallique comprenant au moins un ou plusieurs éléments des terres rares et l'élément fer pour produire un matériau magnétique répondant à la formule générale :
RₓFe_{y}X'ₐZ_{b}
ayant un point de Curie supérieur à 400°C et qui est un composé intermétallique de structure cristalline rhomboédrique ou hexagonale respectivement analogue à Th₂Zn₁₇ et Th₂Ni₁₇, où R représente un ou plusieurs éléments des terres rares, X' est un élément des groupes IIIA, IIIB, IVA ou IVB du tableau périodique des éléments, Z représente un ou plusieurs éléments du groupe VA du tableau périodique des éléments et est incorporé dans les interstices du réseau cristallin dudit composé intermétallique, x est une valeur de 0,5 à 2, y est une valeur de 9 à 19, a est une valeur de 0 à 3, b est une valeur de 0,3 à 3, et Fe est non substitué ou substitué jusqu'à 33 % par un métal de transition, avec la condition que l'élément X' ne soit pas le bore quand le composant Z est l'antimoine ou le bismuth ; ledit procédé comprenant le chauffage dudit composé intermétallique dans un gaz contenant Z, essentiellement en l'absence d'oxygène, pour incorporer Z dans les interstices du réseau cristallin du composé intermétallique au moyen d'une réaction du type gaz-solide.

2. Procédé pour modifier les propriétés magnétiques d'un composé intermétallique comprenant au moins un ou plusieurs éléments des terres rares et l'élément fer pour produire un matériau magnétique répondant à la formule générale :
RₓFe_{y}Z_{b}
ayant un point de Curie supérieur à 400°C et qui est un composé intermétallique de structure cristalline tétragonale analogue à ThMn₁₂, où R représente un ou plusieurs éléments des terres rares, Z représente un ou plusieurs éléments du groupe VA du tableau périodique des éléments et est incorporé dans les interstices du réseau cristallin dudit composé intermétallique, x est une valeur de 0,5 à 2, y est une valeur de 9 à 19, b est une valeur de 0,3 à 3, et Fe est partiellement substitué par un élément du groupe IIIA ou IVA du tableau périodique des éléments ou par un métal de transition provenant d'un autre groupe, le taux de substitution de Fe par n'importe quel métal de transition valant jusqu'à 33 % ; ledit procédé comprenant le chauffage dudit composé intermétallique dans un gaz contenant Z, essentiellement en l'absence d'oxygène, pour incorporer Z dans les interstices du réseau cristallin du composé intermétallique au moyen d'une réaction du type gaz-solide.

3. Procédé tel que revendiqué dans la revendication 1 ou la revendication 2, dans lequel le gaz est un gaz qui produit des radicaux contenant des atomes individuels de l'élément Z du groupe VA par contact avec des surfaces chaudes tel qu'un métal ou le quartz ou par exposition à un rayonnement à haute fréquence.

4. Procédé tel que revendiqué dans la revendication 3, dans lequel le gaz est un hydrure gazeux de l'élément Z du groupe VA.

5. Procédé tel que revendiqué dans la revendication 3, dans lequel l'élément Z du groupe VA est l'azote, et le gaz est l'azote, l'ammoniac ou l'hydrazine.

6. Procédé tel que revendiqué dans l'une quelconque des revendications 1 à 5, dans lequel ledit composé intermétallique est chauffé à une température ne dépassant pas 650°C.

7. Procédé tel que revendiqué dans l'une quelconque des revendications 1 à 6, dans lequel ledit composé intermétallique est broyé jusqu'à l'obtention d'une dimension de particules de 1 à 50 µm de diamètre.

8. Procédé tel que revendiqué dans la revendication 7, dans lequel ledit composé broyé est chauffé pendant une durée allant jusqu'à 8 heures.

9. Procédé tel que revendiqué dans l'une quelconque des revendications précédentes, où R est le samarium ou le néodyme.

10. Procédé tel que revendiqué dans l'une quelconque des revendications 1 et 3, où R est le samarium.

11. Procédé tel que revendiqué dans l'une quelconque des revendications 1 et 3 à 8, où R est le samarium combiné avec un ou plusieurs éléments des terres rares, choisis parmi l'yttrium, le lanthane, le cérium, le néodyme, l'erbium, le thulium et le mischmétal.

12. Procédé tel que revendiqué dans l'une quelconque des revendications 1 et 3 à 8, où R est l'yttrium, le lanthane, le cérium, le praséodyme, le néodyme, le gadolinium, le terbium, le dysprosium, l'erbium, le thulium, l'ytterbium ou le lutétium, ou un mélange d'au moins deux de ces éléments.

13. Procédé tel que revendiqué dans l'une quelconque des revendications 2 à 8, où R est l'yttrium, le thorium, le cérium, le praséodyme, le néodyme, le terbium, le dysprodium ou l'holmium, ou un mélange d'au moins deux de ces éléments.

14. Procédé tel que revendiqué dans la revendication 1 ou l'une quelconque des revendications 3 à 12, où le métal de transition est le cobalt.

15. Procédé tel que revendiqué dans l'une quelconque des revendications 2 à 8 et 13, où l'élément Fe est partiellement substitué par du titane, du vanadium, du molybdène ou du chrome.

16. Procédé tel que revendiqué dans l'une quelconque des revendications 2 à 8 et 13, où l'élément Fe est partiellement substitué par de l'aluminium ou du silicium.

17. Procédé tel que revendiqué dans l'une quelconque des revendications 1 et 3 à 12, où X' est le carbone, le bore, le silicium ou le zirconium, et a est une valeur de 0,1 à 3.

18. Procédé tel que revendiqué dans la revendication 16, où a+b ≤ 3.

19. Procédé tel que revendiqué dans l'une quelconque des revendications précédentes, où Z est l'azote.

20. Procédé tel que revendiqué dans l'une quelconque des revendications 1 à 18, où Z est une combinaison de l'azote avec un ou plusieurs autres éléments du groupe VA.

21. Procédé tel que revendiqué dans l'une quelconque des revendications 1 à 18, où le composant Z représente un ou plusieurs éléments choisis parmi P, As, Sb et Bi.

22. Utilisation du matériau magnétique préparé au moyen du procédé tel que revendiqué dans l'une quelconque des revendications précédentes pour la fabrication d'un aimant permament.

23. Procédé de fabrication d'un aimant permanent à partir d'un matériau magnétique préparé au moyen du procédé selon l'une quelconque des revendications 1 à 21, comprenant les étapes consistant à :
a) broyer ledit matériau magnétique avec un métal tel que l'aluminium, le cuivre ou le zinc ou une poudre organique ou une résine,
b) créer un alignement magnétique dans ledit matériau en appliquant un champ magnétique, et
c) chauffer le produit broyé à une température suffisamment basse pour empêcher la décomposition du matériau magnétique.

24. Procédé tel que revendiqué dans la revendication 23, où, dans le procédé de fabrication de l'aimant, le matériau magnétique est broyé avec 5 à 20 % en poids de zinc.

25. Aimant permanent comprenant un matériau magnétique qui est produit au moyen du procédé tel que revendiqué dans l'une quelconque des revendications 1 à 21.
